

1,264,998.

J. THAME.  
MANUFACTURE OF PAPER YARN.  
APPLICATION FILED FEB. 11, 1915.

Patented May 7, 1918.

2 SHEETS—SHEET 1.



Attest:

Ewd R. Tolson  
Bessie L. Bishop



*Inventor:*

James Thame,  
by Mu Wallace Maffett

1,264,998.

J. THAME.  
MANUFACTURE OF PAPER YARN.  
APPLICATION FILED FEB. 11, 1915.

Patented May 7, 1918.

2 SHEETS—SHEET 2.



Fig. 3.



refig: A.

Attest,

Ewd L. Tolson,  
Bessie L. Bishop

Inventor:

James Thame,  
by Wm Wallace White Atty.

# UNITED STATES PATENT OFFICE.

JAMES THAME, OF LONDON, ENGLAND.

## MANUFACTURE OF PAPER YARN.

1,264,998.

Specification of Letters Patent.

Patented May 7, 1918.

Application filed February 11, 1915. Serial No. 7,654.

To all whom it may concern:

Be it known that I, JAMES THAME, a subject of the King of Great Britain and Ireland, residing at London, England, have 5 invented new and useful Improvements in the Manufacture of Paper Yarn, of which the following is a specification.

This invention relates to the manufacture of paper yarn and has for its object the production of the said yarn in a simple, efficient, and expeditious manner.

This invention consists in the process of producing paper yarn as hereinafter described.

15 To carry the invention into effect I take paper pulp, preferably that known as long stuff, which I feed on to the wet end of a paper making machine. During the feeding of the pulp upon the machine, it is divided into streams of the desired width say for example from 5 to 20 millimeters by means of suitable devices fixed at and in proximity to the feeding end of the wire apron on the paper making machine.

25 Each stream is kept to the desired width during its travel on the wire apron by means of suitably shaped deckles constructed as an endless band and traveling in contact with and in the same direction as the wire.

30 After passing over the vacuum box or boxes and the press roll, the streams of pulp which have now become strips of partially dry paper are fed between felt covered rolls. The bottom roll is made to revolve with and 35 at the same peripheral speed as the top felt covered roll. The effect of this action is to produce a consolidated paper strip which is then twisted in its moist consolidated state and subsequently passed around one or more

40 heated cylinders or equivalently is festooned in a heated drying chamber or arranged to be in contact with heated surfaces for such a time as will enable the material to become sufficiently dry so that it can be twisted upon 45 itself in the form of a yarn. The residual moisture in the twisted yarn can be extracted by passing it over heated cylinders or like devices as it leaves the twisting mechanism and prior to being reeled. In case it

50 is desirable to increase the strength of the paper yarn I simultaneously feed on with the pulp on the wet end of the paper making machine a certain quantity of long fiber such as jute or hemp by means of suitable 55 mechanism in such a way that the long fiber

becomes embedded into and forms part of the paper yarn and this increases its tensile strength.

In order that the invention may be the better understood I will now proceed to describe the same in relation to the accompanying drawings, reference being had to the letters and figures marked thereon. Like letters refer to like parts in the various figures, in which:—

60 Figures 1 and 3, together constitute a diagrammatic side elevation of a machine constructed to carry out my invention.

65 Figs. 2 and 4, are a plan of the machine.

Fig. 5 is a detail view of the dividing 70 devices to an enlarged scale.

Upon an ordinary paper making machine *a* I arrange a series of dividing devices *b* adjacent to the wire apron *c* spaced so as to leave a passage *d* between each pair of devices *b*. The front ends of the devices *b* are wedge shaped and the V-shaped spaces are arranged to be fed with pulp from the stuff box *e* at a uniform level through the orifices *f*, the level being maintained constant by means of an overflow *g*. On the upper side of the wire apron *c* is arranged a number of endless rubber bands or deckles *h* supported by rollers *j* and driven by frictional contact with the wire apron *c*. The 75 series of deckles *h* are mounted a certain distance apart and are of such a width that they just pass between plates *l* mounted on the sides of the dividing devices *b*. Where the deckles *h* and wire apron *c* meet one 80 another the plates *l* form a channel and prevent the pulp from passing between the outer part of the deckles *h* and the wire apron *c*, and at the same time train the stream of pulp drawn in by the co-active 85 relationship of the wire apron *c* and deckles *h* and thus insure the stream of pulp having a uniform solid constituent. After passing over the vacuum box *m* and from between the deckles *h* the now consolidated pulp 90 strips pass under the press roll *n* and delivery felt covered rollers *o* to a twisting machine *p*, along a drying device such as a steam jacketed conical shaped trough *q* to a reeling machine *r*. In case it is desirable 95 to combine some long fiber such as jute or hemp with the pulp to strengthen the tensile resistance of the resultant yarn I embed the long fiber in a matrix of pulp. I arrange at the front end of the machine *a* some 100

105 long fiber such as jute or hemp with the pulp to strengthen the tensile resistance of the resultant yarn I embed the long fiber in a matrix of pulp. I arrange at the front end of the machine *a* some 110

form of device which will feed into each of the pulp streams a regulated weight of long fiber, for example; an endless band *s* driven at a constant lineal speed has a definite amount of the long fibers either hand or mechanically spread over a unit of its length, this strip of material formed wholly of long fibers is fed between the rollers *t* and consolidated thereby. Rollers *u* are provided and driven at such rate which shall be at least equal to the lineal speed of the wire apron *c* and in excess of the velocity of the rollers *t* that they produce a drawing action of the material between them and the said rollers *t*. Between the rollers *t* and the rollers *u* knives *v* are arranged to split the web of material into a given number of strands *w* which after passing through the rollers *u* are led around rollers *x* and *x'* and thereby diverted into the stream of pulp, rollers *y* and *y'* being provided to press and maintain the strands in their correct positions.

In order that the quantity of long fiber fed on to the endless band *s* may be regulated, the movements of the said band *s* are indicated on the dial *z* the pointer of which is rotated by means of a chain or the like *z'* running on and being driven by a sprocket

mounted on one of the rollers carrying the 30 said band *s*.

Although the knives *v* shown in the drawing are of the rotary type it is obvious I may use parting knives of a stationary or reciprocating character if desired. 35

I claim:—

The method of manufacturing reinforced paper yarn which consists in simultaneously feeding a mass of pulp and relatively long vegetable fibers onto the intake end of a 40 paper making machine, dividing the mass at or adjacent to its point of entry into a series of streams, maintaining the streams separated throughout their passage through the machine to produce a number of narrow 45 paper bands having deckle edges, subjecting the bands to pressure to consolidate them and to incorporate the fiber therewith, twisting the bands into round threads, and finally drying the product.

In testimony whereof I have signed my name to this specification in the presence of two subscribing witnesses.

JAMES THAME.

Witnesses:

R. W. JAMES,  
CHAS. R. BALLOUGH.